# EUROPEAN PATENT SPECIFICATION

(11) **EP 0 324 426 B1**
(45) Date of publication and mention of the grant of the patent: **19.06.1996**
(21) Application number: 89100317.0
(22) Date of filing: 10.01.1989
(51) Int. Cl.: G03C 1/10

(54) **Process for forming super high contrast negative images**
Verfahren zur Erzeugung von extrem hochkontrastreichen negativen Bildern
Procédé pour former des images négatives à très haut contraste

(30) Priority: 11.01.1988 JP 3445/88; 11.01.1988 JP 3446/88
(43) Date of publication of application: 19.07.1989
(73) Proprietor: FUJI PHOTO FILM CO., LTD., Kanagawa 250-01 (JP)
(72) Inventor: Takagi, Yoshihiro c/o Fuji Photo Film Co., Ltd., Minami Ashigara-shi Kanagawa (JP); Okada, Hisashi c/o Fuji Photo Film Co., Ltd., Minami Ashigara-shi Kanagawa (JP); Yagihara, Morio c/o Fuji Photo Film Co., Ltd., Minami Ashigara-shi Kanagawa (JP)
(74) Representative: Patentanwälte Dr. Solf & Zapf

(56) References cited:
- EP-A- 0 249 239
- JP-A- 6 230 243
- RESEARCH DISCLOSURE. vol. 236, December 1983, HAVANT GB pages 382 - 383; R. Pollet et al.: "Benzamin:Preparation and use as stabilizers in silver halide materials of bidentate heterocyclic compounds containing an aminogroup"

## Description

### FIELD OF THE INVENTION

This invention relates to a silver halide photographic material and a process for forming super high contrast negative images. More particularly, the invention relates to a silver halide photographic material for use in a photomechanical process.

### BACKGROUND OF THE INVENTION

In the field of graphic arts, an image forming system having super high contrast (in particular, a gamma ($\overline{\text{G}}$) of at least 10) is required for improving the reproduction of continuous tone by dot images or the reproduction of line images.

For this purpose, a specific developer called "lith developer" has hitherto been used. The lith developer consists of hydroquinone as the developing agent and also contains a sulfite as a preservative in the form of an addition product with formaldehyde, whereby the concentration of free sulfite ions is reduced as low as possible (typically below 0.1 mol/liter). Accordingly, the lith developer is susceptible to air-oxidation and thus cannot be stored for over 3 days.

Methods of obtaining high contrast and high sensitivity photographic characteristics using a stable developer and hydrazine derivatives are described in US-A-4,224,401, 4,168,977, 4,166,742, 4,311,781, 4,272,606, 4,211,857, and 4,243,739. Furthermore since sulfite can be added at a high concentration, the stability of the developer to air oxidation is greatly improved as compared to the lith developer.

However, for forming super high contrast images using a hydrazine derivative, the pH of the developer must be at least 11.0. In such circumstances, the developing agent is liable to be oxidized, the pH is liable to deviate by absorbing CO₂ from the air and stable photographic properties are thus not obtained. Accordingly, a process of obtaining super high contrast images in a developer having a high sulfite ion concentration at a pH below 11.0 has been desired.

A means for increasing the activity of hydrazine has been keenly desired and in this regard, phosphonium salt compounds in JP-A-61-167939 (the term "JP-A" as used herein mean as "unexamined published Japanese patent application"), disulfide compounds in JP-A-61-198147, and amine series compounds in JP-A-60-140340 are disclosed as contrast enhancing agents. However, even by using these compounds, it is difficult to further enhance contrast at a pH below 11.

On the other hand, a low-speed, light-sensitive material for safelight use employing a hydrazine compound, and containing a water-soluble rhodium salt, is disclosed in JP-A-60-83038 and 60-162246. However, in this case, the addition of a sufficient amount of rhodium salt to increase the sensitivity obstructs the increase of contrast by the hydrazine compound, whereby the desired sufficiently high contrast images are not obtained.

JP-A-62 030 243 discloses a silver halide photographic material comprising a support having provided thereon at least one silver halide emulsion layer, wherein said emulsion layer or another layer of the silver halide photographic material provided on the support contains at least one compound represented by the following formula (I) and at least one blocked development restrainer represented by the following formula (II), and a process for forming a super-high contrast negative image comprising imagewise exposing the above-described photographic material to light and developing the exposed material with a developer containing not less than 0.15 mol/l of a sulfite ion and having a pH of from 10.5 to 12.3. wherein A represents an aliphatic group or an aromatic group; B represents a formyl group, an acyl group, an alkyl- or arylsulfonyl group, an alkyl- or arylsulfinyl group, a carbamoyl group, an alkoxy- or aryloxycarbonyl group, a sulfinamoyl group, an alkoxysulfonyl group, a thioacyl group, a thiocarbamoyl group or a heterocyclic group; R₀ and R₁ each represents a hydrogen atom, a substituted or unsubstituted alkylsulfonyl group, a substituted or unsubstituted arylsulfonyl group or a substitued or unsubstituted acyl group, with the proviso that at least one of R₀ and R₁ is a hydrogen atom; and B, R₁ and the nitrogen atom to which B and R₁ are bonded may jointly form -N=C< (a partial structure of hydrazone).

C_{A} - D (II)

wherein C_{A} represents a blocking group capable of releasing a development restrainer or a precursor thereof at the time of development processing regardless of the exposure amount; and D represents a development restrainer or a precursor thereof that is bonded to C_{A} via a hetero atom of D. The development processing of this known silver halide photographic material is carried out with a developer having a pH of 11.6.

### SUMMARY OF THE INVENTION

An object of this invention, therefore, is to provide a process of forming super high contrast images using a developer having a pH of from 9.6 to 11.0 in a system containing a hydrazine compound.

Another object of this invention is to provide a process of forming super high contrast images with stable photographic performance using a stable developer.

It has now been discovered that the aforesaid objectives can be attained by the process of the present invention as set forth below.

The present invention provides a process for forming super high contrast negative images, which comprises processing a super high contrast negative type silver halide photographic material comprising a support having thereon at least one layer, one of which must be a silver halide emulsion layer, said silver halide emulsion layer or other hydrophilic colloid layer containing at least one hydrazine derivative and at least one nucleation accelerator represented by following formula (Ia) or (Ib) with a developer having a pH of from 9.6 to less than 10.5;

M₁S(̵X)̵ₙA₃-B (Ib)

wherein Y represents a group adsorbing onto silver halide; A₁ represents a divalent linkage group composed of an atom or an atomic group selected from carbon, nitrogen, oxygen, and sulfur; A₂ represents a divalent linkage group; A₃ represents a linkage group composed of an atom or an atomic group selected from carbon, nitrogen, oxygen, and sulfur; B represents a substituted or unsubstituted amino group, an ammonium group, or a nitrogen-containing heterocyclic ring; X represents a divalent heterocyclic ring containing nitrogen, oxygen, selenium or sulfur; M₁ represents a hydrogen atom, an alkali metal, an alkaline earth metal, a quaternary ammonium salt, a quaternary phosphonium salt, an amidino group; m represents the integer of 1, 2 or 3; and n and p each represents 0 or the integer 1.

### DETAILED DESCRIPTION OF THE INVENTION

The compounds for use in the present invention are described in detail.

In formula (Ia) described above, Y represents a group which adsorbs onto silver halide as, for example, a nitrogen-containing heterocyclic group.

When Y represents a nitrogen-containing heterocyclic group, the compound of formula (Ia) is shown by formula (II) wherein ℓ represents 0 or the integer 1; [(A₁)̵_{P}A₂-B]ₘ has the same meaning as in formula (Ia) described above; and Q represents an atomic group necessary for forming a 5-or 6-membered heterocyclic ring composed of members selected from carbon, nitrogen, oxygen, and sulfur. R the condensation product of said 5- or 6-membered ring with a carbon aromatic ring or a heteroaromatic ring; M₂ represents hydrogen, an alkali metal atom, an ammonium group or a group capable of being replaced with hydrogen or an alkali metal atom under alkali conditions.

Examples of the heterocyclic ring formed by Q include the indazoles, benzimidazoles, benzotriazoles, benzoxazoles, benzthiazoles, imidazoles, thiazoles, oxazoles, triazoles, tetrazoles, azaindenes, pyrazoles, indoles, triazines, pyrimidines, pyridines, and quinolines. These heterocyclic rings may be substituted as indicated below.

In formula (II) examples for the alkali metal atom in M₂ are sodium and potassium, for an ammonium group, e.g. trimethylammonium and dimethylbenzylammonium, or for a group capable of being replaced with hydrogen or an alkali metal atom under alkali conditions, e.g. acetyl, cyanoethyl, and methanesulfonylethyl.

Also, these heterocyclic rings may be substituted by a nitro group, a halogen atom (e.g., chlorine and bromine), a mercapto group, a cyano group, a substituted or unsubstituted alkyl group (e.g., methyl, ethyl, propyl, t-butyl cyanoethyl, methoxyethyl, and methylthioethyl), a substituted or unsubstituted aryl group (e.g., phenyl, 4-methanesulfonamidophenyl, 4-methylphenyl, 3,4-dichlorophenyl, and naphthyl), a substituted or unsubstituted alkenyl group (e.g., allyl), a substituted or unsubstituted aralkyl group (e.g., benzyl, 4-methylbenzyl, and phenethyl), a substituted or unsubstituted alkoxy group (e.g., methoxy and ethoxy), a substituted or unsubstituted aryloxy group (e.g., phenoxy and 4-methoxyphenoxy), a substituted or unsubstituted alkylthio group (e.g., methylthio, ethylthio, and methoxyethylthio), a substituted or unsubstituted arylthio group (e.g., phenylthio), a substituted or unsubstituted sulfonyl group (e.g., methanesulfonyl, ethanesulfonyl, and p-toluenesulfonyl), a substituted or unsubstituted carbamoyl group (e.g., unsubstituted carbamoyl, methylcarbamoyl, and phenylcarbamoyl), a substituted or unsubstituted sulfamoyl group (e.g., unsubstituted sulfamoyl, methylsulfamoyl, and phenylsulfamoyl), a substituted or unsubstituted carbonamido group (e.g., acetamido group and benzamido group), a substituted or unsubstituted sulfonamido group (e.g., methanesulfonamido, benzenesulfonamido, and p-toluenesulfonamido), a substituted or unsubstituted acyloxy group (e.g., acetyloxy and benzoyloxy), a substituted or unsubstituted sulfonyloxy group (e.g., methanesulfonyloxy), a substituted or unsubstituted ureido group (e.g., unsubstituted ureido, methylureido, ethylureido, and phenylureido), a substituted or unsubstituted thioureido group (e.g., unsubstituted thioureido and methylthioureido), a substituted or unsubstituted acyl group (e.g., acetyl and benzyl), a substituted or unsubstituted heterocyclic group (e.g., 1-morpholino, 1-piperidino, 2-pyridyl, 4-pyridyl, 2-thienyl, 1-pyrazolyl, 1-imidazolyl, 2-tetrahydrofuryl, and tetrahydrothienyl), a substituted or unsubstituted oxycarbonyl group (e.g., methoxycarbonyl and phenoxycarbonyl), a substituted or unsubstituted oxycarbonylamino group (e.g., methoxycarbonylamino, phenoxycarbonylamino, and 2-ethylhexyloxycarbonylamino), a substituted or unsubstituted amino group (e.g., unsubstituted amino, dimethylamino, methoxyethylamino, and anilino), a carboxylic acid or a salt thereof, a sulfonic acid or a salt thereof, and a hydroxy group.

Examples of the divalent linkage group shown by A₁ include:

In the above formulae, R₁, R₂, R₃, R₄, R₅, R₆, R₇, R₈, R₉, and R₁₀ each represents a hydrogen atom, a substituted or unsubstituted alkyl group (e.g., methyl, ethyl, propyl, and n-butyl), a substituted or unsubstituted aryl group (e.g., phenyl and 2-methylphenyl), a substituted or unsubstituted alkenyl group (e.g., propenyl and 1-methylvinyl), or a substituted or unsubstituted aralkyl group (e.g., benzyl and phenethyl).

The above divalent structures may be further combined with a straight chain or branched alkylene group preferably having to 1 to 6 carbon atoms and more preferably 1 to 3 carbon atoms (e.g., methylene, ethylene, propylene, butylene, hexylene, and 1-methylethylene) to also comprise A₁, e.g.

In formula (II), A₂ represents a divalent linkage group such as a straight chain or branched alkylene group (e.g., methylene, ethylene propylene, butylene, hexylene, and 1-methylethylene), a straight chain or branched alkenylene group (e.g., vinylene and 1-methylvinylene), a straight chain or branched aralkylene group (e.g., benzylidene), a straight chain or branched arylene group (e.g., phenylene and naphthylene).

A₁ and A₂ in formula (II) may be further substituted with the groups represented by A₁ and A₂.

The substituted or unsubstituted amino group shown by B in formula (II) is shown by formula (VII). wherein R¹¹ and R²², which may be the same or different, each represents a hydrogen atom, a substituted or unsubstituted alkyl, alkenyl group or aralkyl group having from 1 to 30 carbon atoms and these groups may be straight chain groups (e.g., methyl, ethyl, n-propyl, n-butyl, n-octyl, allyl, 3-butenyl, benzyl, and 1-naphthylmethyl), branched groups (e.g., iso-propyl and t-octyl), or cyclic groups (e.g., cyclohexyl).

Also, R¹¹ and R¹² may combine with each other to form a ring which may contain at least one hetero atom (e.g., oxygen, sulfur and nitrogen) so as to form a saturated heterocyclic ring such as pyrrolidyl, piperidyl and morpholino.

Furthermore, substituents for R¹¹ and R¹² include a carboxy group, a sulfo group, a cyano group, a halogen atom (e.g., fluorine, chlorine, and bromine), a hydroxy group, an alkoxycarbonyl group having from 1 to 20 carbon atoms (e.g., methoxycarbonyl, ethoxycarbonyl, phenoxycarbonyl, and benzyloxycarbonyl), an alkoxy group having from 1 to 20 carbon atoms (e.g., methoxy, ethoxy, benzyloxy, and phenetyloxy), an aryloxy group having not more than 20 carbon atoms (e.g., phenoxy and p-tolyloxy), an acyloxy group having not more than 20 carbon atoms (e.g., acetyloxy and propionyloxy), an acyl group having not more than 20 carbon atoms (e.g., acetyl, propionyl, benzoyl, and mesyl), a carbamoyl group (e.g., carbamoyl, N,N-dimethylcarbamoyl, morpholinocarbonyl, and piperidinocarbonyl), a sulfamoyl group (e.g., sulfamoyl, N,N-dimethyIsuIfamoyI, morpholinosulfonyl, and piperidinosulfonyl), an acylamino group having not more than 20 carbon atoms (e.g., acetylamino, propionylamino, benzoylamino, mesylamino), a sulfonamido group (e.g., ethylsulfonamido and p-toluenesulfonamido), a carbonamido group having not more than 20 carbon atoms (e.g., methylcarbonamido and phenylcarbonamido), a ureido group having not more than 20 carbon atoms (e.g., methylureido and phenylureido), an amino group (same ones as defined in formula (VII)).

The ammonium group shown by B is generally shown by formula (VIII). wherein R¹³, R¹⁴, and R¹⁵ have the same meaning as R¹¹ and R¹² in formula (VII) as described above and Z^{⊖} represents an anion such as halide ion (e.g., Cl^{⊖}, Br^{⊖} and I^{⊖} ) a sulfonate ion (e.g., trifluoromethanesulfonate ion, p-toluenesulfonate ion, benzenesulfonate ion, and pchlorobenzenesulfonate ion), a sulfate ion (e.g., ethyl sulfate ion and methyl sulfate ions), a prechlorate ion, a tetrafluoroborate ion and Also, q represents the integer 0 or 1 and when the compound forms an intramolecular salt, q is 0.

As a nitrogen-containing heterocyclic ring, B is a 5- or 6-membered ring containing at least one nitrogen atom and the ring may have substituents or may be condensed with another ring. Examples of the nitrogen containing heterocyclic ring are an imidazolyl ring, a pyridyl ring, and a thiazolyl ring.

Preferred embodiments of formula (II) are shown by formulae (III), (IV), (V), or (VI); wherein (A₁)p-A₂-B, M₂ and m have the same meaning as defined above in formula (II); Z₁, Z₂, and Z₃ have the same meaning as (A₁)̵_{P}A₂-B in formula (Ia) or each represents a halogen atom, an alkoxy group having from 1 to 20 carbon atoms (e.g., methoxy), a hydroxy group, a hydroxyamino group, or a substituted or unsubstituted amino group. The substituent for the amino group can be selected from the aforesaid substituents for R¹¹ and R¹² in formula (VII). At least one of Z₁, Z₂, and Z₃ must have the same meaning as (A₁)̵ₚA₂-B.

These heterocyclic rings may be substituted by the substituents applied to the heterocyclic ring shown by Q in formula (II) as described above.

The heterocyclic ring shown by X in formula (Ib) described above is a 5- or 6-membered heterocyclic ring containing at least one of nitrogen, oxygen, selenium, and sulfur and may be condensed with a carbon aromatic ring or a hetero aromatic ring. The heterocyclic ring is preferably aromatic and examples thereof are tetrazole, triazole, thiadiazole, oxadiazole, selenadiazole, imidazole, thiazole, oxazole, benzimidazole, benzthiazole, benzoxazole, benzselenazole, and pyrimidine. Among them, tetrazole and thiazole are particularly preferred.

These heterocyclic rings may be substituted by the same substituents applied to the heterocyclic rings shown by Q in formula (II).

The divalent linkage group shown by A₃ in formula (Ib) is a divalent linkage group composed of an atom or an atomic group selected from hydrogen, carbon, nitrogen, oxygen, and sulfur. Examples thereof are those illustrated as the linkage groups of A₁ and A₂ in formula (Ia) and a straight chain or branched alkinylene group (e.g., -CH-C≡C-CH-). The linkage group shown by A₃ may further comprise a linkage group by combinations of A₁, A₂ and/or an alkinylene group , e.g.,

The alkali metal shown by M₁ in formula (Ib) includes Na⁺, K⁺, and Li⁺. The alkaline earth metal shown by M₁ includes Ca⁺⁺, and Mg⁺⁺. The quaternary ammonium salt shown by M₁ has from 4 to 30 carbon atoms and examples thereof include, (CH₃)₄N^{⊕}, (C₂H₅)₄N^{⊕}, (C₄H₉)₄N^{⊕}, C₆H₅CH₂N^{⊕}(CH₃)₃, and C₁₆H₃₃N^{⊕}(CH₃)₃. Also, examples of the quaternary phosphonium salt include (C₄H₉)₄P^{⊕} , C₁₆H₃₃P^{⊕}(CH₃)₃, and C₆H₅CH₂P^{⊕}(CH₃)₃.

The group shown by M1, which can be replaced with hydrogen or an alkali metal atom under alkali conditions include an acetyl group, a cyanoethyl group, and a methanesulfonylethyl group.

Specific examples of the compound shown by formula (Ia) are illustrated below but the invention is not limited to these examples.

Specific examples of the compound of formula (Ib) are illustrated below but the invention is not limited to these compounds. $\text{Ib-45} {\text{(HOCH}}_{\text{2}} {\text{CH}}_{\text{2}} {\text{)}}_{\text{2}} {\text{NCH}}_{\text{2}} {\text{CH}}_{\text{2}} \text{SH}$

The nucleation accelerators shown by formulae (Ia) and (Ib) are readily synthesized by the methods described in Berichte der Deutschen Chemischen Gesellschaft, 28, 77(1895), ibid., 22, 568 (1889), ibid., 29, 2483(1896), Journal of Chemical Society, 1932, 1806, Journal of The American Chemical Society, 71, 4000(1949), Advances in Heterocyclic Chemistry, 9, 165(1968), Organic Synthesis, IV, 569(1963), Journal of The American Chemical Society, 45, 2390(1923), Chemische Berichte, 9, 465(1976), JP-A-50-37436 and JP-A-51-3231, U.S. Patents 3,295,976, 3,376,310, 2,585,388, and 2,541,9.24, JP-B-40-28496, JP-B-43-41353, JP-B-60-29390, JP-B-60-29391, JP-B-60-133061, and JP-B-61-1431 (the term "JP-B" as used herein means an "examined published Japanese patent application"), US-A-3,106,467, 3,420,670, 2,271,229, 3,137,578, 3,148,066, 3,511,663, 3,060,028, 3,271,154, 3,251,691, 3,598,599, 3,148,066, 3,615,616, 3,420,664, 3,071,465, 2,444,605, 2,444,606, 2,444,607, and 2,935,404, and JP-A-50-89034, JP-A-57-202531, JP-A-57-167023, JP-A-57-164735, JP-A-60-80839, JP-A-58-152235, JP-A-57-14836, JP-A-59-162546, JP-A-60-130731, JP-A-60-138548, JP-A-58-83852, JP-A-58-159529, JP-A-59-159162, JP-A-60-217358, and JP-A-61-80238.

These accelerators may be used singly or in combination thereof.

The hydrazine derivative for use in the present invention includes those having a sulfinyl group as described in US-A-4,478,928 and the compound shown by formula (IX).

R₂₁-NHNH-CHO (IX)

wherein R₂₁ represents an aliphatic group or an aromatic group.

The aliphatic group shown by R₂₁ in formula (IX) is preferably an aliphatic group having from 1 to 30 carbon atoms. A straight chain, branched, or cyclic alkyl group having from 1 to 20 carbon atoms is preferred. The branched alkyl group may be cyclized so as to form a saturated heterocyclic ring containing at least one hetero atom. Also, the aforesaid alkyl group may have a substituent such as an aryl group, an alkoxy group, a sulfoxy group, a sulfonamido group, and a carbon-amido group.

Examples thereof are t-butyl, n-octyl, t-octyl, cyclohexyl, pyrrolidyl, imidazolyl, tetrahydrofuryl, and morpholino.

The aromatic group shown by R₂₁ in formula (IX) is a monocyclic or dicyclic aryl group or an unsaturated heterocyclic group. The unsaturated heterocyclic group may be condensed with a monocyclic or dicyclic aryl group to form a heteroaryl group.

Examples thereof are a benzene ring, a naphthalene ring, a pyridine ring, a pyrimidine ring, an imidazole ring, a pyrazole ring, a quinoline ring, an isoquinoline ring, a benzimidazole ring, a thiazole ring, and a benzothiazole ring. Among them, the groups having a benzene ring are preferred.

R₂₁ is a particularly preferred aryl group.

The aryl group or aromatic group shown by R₂₁ may be substituted. Typical examples of the substituent include a straight chain, branched, or cyclic alkyl group (preferably having from 1 to 20 carbon atoms), an aralkyl group (preferably a monocyclic or dicyclic ring the alkyl moiety of which has from 1 to 3 carbon atoms), an alkoxy group (preferably having from 1 to 20 carbon atoms), a substituted amino group (preferably an amino group substituted by an alkyl group having from 1 to 20 carbon atoms), an acylamino group (preferably having from 2 to 30 carbon atoms), a sulfonamido group (preferably having from 1 to 30 carbon atoms) and a ureido group (preferably having from 1 to 30 carbon atoms).

R₂₁ in formula (IX) may have therein a ballast group being usually used to immobilize photographic additives such as couplers, etc. The ballast group is a group having at least 8 carbon atoms and is relatively inert to photographic properties. Examples thereof include an alkyl group, an alkoxy group, a phenyl group, an alkylphenyl group, a phenoxy group, and an alkylphenoxy group.

R₂₁ in formula (IX) may have therein a group for enhancing the adsorption onto the surface of silver halide grains. Such adsorptive groups include a thiourea group, a heterocyclic thioamido group, a mercaptoheterocyclic group, a triazole group, as disclosed in US-A-4,385,108.

Synthesis methods for the compounds shown by formula (IX) are disclosed in JP-A-53-20921, JP-A-53-20922, JP-A-53-66732 and JP-A-53-20318.

Specific examples of the compound shown by formula (IX) are illustrated below, but the invention is not limited to these compounds.

Other examples of the compound shown by formula (IX) are the following compounds disclosed in US-A-4,478,928.

In the present invention, particularly preferred compounds of formula (IX) have therein a group which enhances adsorption onto the surface of silver halide grains. Such adsorptive groups include a thiourea group, a heterocyclic thioamido group, a mercaptoheterocyclic group, and a triazole group as disclosed in US-A-4,385,108. The preferred substituents for the aryl group or aromatic group shown by R₁ include an amido group, a ureido group, and a thiourea group. A sulfonamido group is particularly preferred.

The nucleation accelerator and the hydrazine derivative of the present invention are preferably incorporated in a silver halide emulsion layer, but they may also be incorporated in other light-insensitive hydrophilic colloid layers (e.g., protective layer, interlayer, filter layer, and antihalation layer), preferably those adjacent to a silver halide emulsion layer. They may be added in the same layer or different layers. Water soluble compound of formulae(Ia), (Ib) and (IX) may be added to the hydrophilic colloid solution as an aqueous solution thereof. Conversly, when the compound is sparingly soluble in water, the compound may be added thereto as a solution in an organic solvent which is miscible with water. Examples of solvent include water, methanol, ethanol, acetone, dimethylformamide, and methylcellosolve. When the compound of formula (Ia), (Ib) or (IX) is incorporated into the silver halide emulsion layer, the addition may be performed at any optional time from the initiation of chemical ripening to just prior to coating, but the compound is preferably added thereto after chemical ripening is complete and prior to coating. It is particularly preferred to add the compound to the coating composition prepared for coating.

The optimal amount of the compounds of formula (Ia), (Ib) and (IX) are selected according to the grain size and the halogen composition of the silver halide emulsion, the method and extent of chemical sensitization, the relation -between the layer(s) in which the compounds are incorporated and a silver halide emulsion, and the kind of an antifoggant.

The addition amount of the compound of formula (Ia) for use in the present invention is preferably from 5 mg/m² to 500 mg/m², and 10 mg/m² to 250 mg/m² is particularly preferred. Also, the addition amount of the compound of formula (Ib) is preferably from 1 mg/m² to 250 mg/m², and 3 mg/m² to 150 mg/m² is particularly preferred. Furthermore, the addition amount of the compound of formula (IX) is preferably from 1 mg/m² to 300 mg/m², and 2 mg/m² to 200 mg/m² is particularly preferred. Also, the compound of formula (IX) wherein R₂₁ contains therein a group enhancing the adsorption onto the surface of silver halide grains is preferably added in an amount of from 2 mg/m² to 100 mg/m².

The photographic emulsion for use in the present invention may contain silver bromide, silver iodobromide, silver iodochlorobromide, silver chlorobromide, silver iodide, or silver chloride, but it is preferred that the silver halide contains at least 50 mol% silver chloride.

The silver halide grains in the photographic emulsion may have a regular crystal form such as cubic, octahedral, dodecahedral, and tetradecahedral; an irregular crystal form such as sphere, and tabular; or a composite of these crystal forms. The silver halide grains may be composed of a mixture of grains having various crystal forms.

The silver halide grains for use in the present invention may have different phase between the inside and the surface layer thereof or may be composed of a uniform phase throughout the whole grain.

During the During the formation or physical ripening of the silver halide grains, a cadmium salt, a zinc salt, a lead salt, a thallium salt, an iridium salt or a complex salt thereof, rhodium salt or a complex salt thereof, iron salt or a complex salt thereof, etc., may be present in the system.

Also, a silver halide solvent (e.g., ammonia, potassium rhodanate, and thioethers and thione compounds as described in US-A-3,271,157, JP-A-51-12360, JP-A-53-82408, JP-A-53-144319, JP-A-54-100717, and JP-A-54-155828) can be used as required in the present invention.

The silver halide emulsion for use in the present invention may or may not be chemically sensitized. Chemical sensitization for use in the present invention include a sulfur sensitization method using active gelatin or a sulfur-containing compound capable of reacting with silver (e.g., thiosulfates, thioureas, mercapto compounds, and rhodanines); a reduction sensitizing method using a reducing material (e.g., stannous salt, amines, hydrazine derivatives, formamidinesulfinic acid, and silane compounds); a noble metal sensitization method using a metal compound (e.g., gold complex salts and complex salts of noble metals belonging to group VIII of the Periodic Table, such as Pt, Ir, and Pd); or a combination thereof.

The silver halide emulsions for use in this invention can contain various compounds for preventing the formation of fog during the storage and/or photographic processing of the light-sensitive material or for stabilizing photographic performance. For example, such antifoggants or stabilizers include azoles (e.g., benzothiazoliums, nitroindazoles, triazoles, benzotriazoles, benzimidazoles (in particular, nitro- or halogen-substituted benzimidazoles)); heterocyclic mercapto compounds (e.g., mercaptothiazoles, mercaptobenzothiazoles, mercaptobenzimidazoles, mercaptothiadiazoles, mercaptotetrazoles (in particular, l-phenyl-5-mercaptotetrazole), and mercaptopyrimidines), the aforesaid heterocyclic mercapto compounds having a water-solubilizing group such as a carboxy group and a sulfon group, thioketo compounds (e.g., oxazolinethione), azaindenes (e.g., tetraazaindenes (in particular, 4-hydroxy-substituted (1,3,3a,7)tetraazaindenes), benzenethiosulfonic acids, and benzenesulfinic acid.

The photographic emulsion for use in the present invention may be spectrally sensitized to relatively a long wavelength of blue light, green light, red light, or infrared light using sensitizing dyes. Such sensitizing dyes include cyanine dyes, merocyanine dyes, complex cyanine dyes, complex merocyanine dyes, holopolar cyanine dyes, styryl dyes, hemicyanine dyes, oxonol dyes, and hemioxonol dyes.

Practical examples of the spectral sensitizing dyes are disclosed in, for example, P. Glafkides, Chemie Photographique, 2nd edition, Chapters 35 to 41, published by Paul Montel, Paris, 1957, F.M. Hamer, The Canine and Related Compound, Interscience, U.S. Patents 2,503,776, 3,459,553, and 3,177,210, and Research Disclosure, Vol. 176, No. 17643, Paragraph 23, IV-J, (December, 1978).

The photographic light-sensitive material being processed in the present invention may contain water-soluble dyes in the hydrophilic colloid layer(s) as filter dyes or for irradiation inhibition, etc. Such dyes include oxonol dyes, hemioxonol dyes, styryl dyes, merocyanine dyes, cyanine dyes and azo dyes. Among them, oxonol dyes, hemioxanol dyes, and merocyanine dyes are particularly useful.

Also, the photographic light-sensitive material of the present invention may further contain in the photographic emulsion layer(s) and other hydrophilic colloid layer(s) an inorganic or organic hardening agent. For example, active vinyl compounds (e.g., 1,3,5-triacryloyl-hexahydro-s-triazine and 1,3-vinylsulfonyl-2-propanol) and active halogen compounds (e.g., 2,4-dichloro-6-hydroxy-s-triazine) can be used singly or as a combination thereof.

Furthermore, the photographic light-sensitive material of the present invention may further contain in the photographic emulsion layer(s) or other hydrophilic colloid layer(s) various surface active agents.

Examples of surface active agent for use in the present invention are nonionic surface active agents such as saponin (steroid series), alkylene oxide derivatives (e.g., polyethylene glycol, polyethylene glycol/polypropylene glycol condensates, polyethylene glycol alkyl ethers, polyethylene glycol alkylaryl ethers, polyethylene glycol esters, polyethylene glycol sorbitan esters, polyalkylene glycol alkylamines, polyalkylene glycol alkylamides, and polyethylene oxide addition products of silicone), glycidol derivatives (e.g., alkenyl succinic acid polyglyceride and alkylphenol polyglyceride), aliphatic acid esters of polyhydric alcohols, alkyl esters of saccharide, etc.; anionic surface active agents containing an acid group (e.g., a carboxy group, a sulfo group, a phospho group, a sulfuric acid ester group, and a phosphoric acid ester group), such as alkyl carboxylates, alkyl sulfonates, alkylbenzenesulfonates, alkylnaphthalenesulfonates, alkylsulfuric acid esters, alkylphosphoric acid esters, N-acyl-N-alkyltaurins, sulfosuccinic acid esters, sulfoalkyl polyoxyethylene alkylphenyl ethers, polyoxyethylene alkylphosphoric acid esters; amphoteric surface active agents such as amino acids, aminoalkylsulfonic acids, aminoalkylsulfuric acid esters, aminoalkylphosphoric acid esters, alkylbetaines, amine oxides, etc.; and cationic surface active agents such as alkylamine salts, aliphatic quaternary ammonium salts, aromatic quaternary ammonium salts, heterocyclic quaternary ammonium salts (e.g., pyridinium and imidazolium), phosphonium or sulfonium salts containing an aliphatic or aromatic ring, etc.

The photographic emulsion layer(s) of the photographic light-sensitive material of the present invention may further contain polyalkylene oxide or the derivatives thereof such as the ethers, esters, amines, etc., thereof, thioether compounds, thiomorpholines, quaternary ammonium salt compounds, urethane derivatives, urea derivatives, imidazole derivatives, and 3-pyrazolidone derivatives for increasing sensitivity, contrast, and/or accelerating development.

As the binder or protective colloid for the emulsion layer(s) and other hydrophilic colloid layer(s) of the photographic light-sensitive material of the present invention, gelatin is advantageously used, but other hydrophilic colloids can also be used.

For example, hydrophilic high molecular materials such as polyvinyl alcohol, polyvinyl alcohol partial acetal, poly-N-vinylpyrrolidone, polyacrylic acid, polyacrylamide, dextran, etc. may be used.

In order to obtain photographic characteristics of super high contrast of the silver halide photographic material formed in the process of the present invention, a stable developer can be used without use of either a conventional infectious developer or a high alkaline developer of about pH 13 as described in US-A-2,419,975.

That is, using the process of the present invention, super high contrast negative images are obtained by processing the light-sensitive material in the present invention with a developer containing a sulfite ion at a concentration of at least 0.15 mol/liter and having pH of from 9.6 to less than 10,5.

There is no particular restriction on the developing agent which can be used in the process of the present invention and, for example, dihydroxybenzenes (e.g., hydroquinone), 3-pyrazolidones (e.g., 1-phenyl-3-pyrazolidone, 4,4-dimethyl-1-phenyl-3-pyrazolidone), and aminophenols (e.g., N-methyl-p-aminophenol) can be used singly or in combination thereof.

The silver halide light-sensitive material in the present invention is preferably processed by a developer containing a dihydroxybenzene as the primary developing agent and a 3-pyrazolidone or an aminophenol as an auxiliary developing agent. In this case, it is preferred that the developer contain the dihydroxybenzene in the range of from 0.05 to 0.5 mol/liter and the 3-pyrazolidone or aminophenol in the range of less than 0.06 mol/liter.

Also, as disclosed in US-A-4,269,929, by adding an amine to the developer, the developing speed can be increased to thus shorten the development time.

The developer for use in the present invention may further contain pH buffers such as sulfites, carbonates, borates, and phosphates of an alkali metal or a development inhibitors or antifoggants such as bromides, iodides and organic antifoggants (nitro-indazoles or benzotriazoles are particularly preferred). Also, if necessary, the developer may contain a water softener, a resolution aid, a toning agent, a development accelerator, a surface active agent (a polyalkylene oxide is particularly preferred), a defoaming agent, a hardening agent, and/or a silver stain inhibitor of films (e.g., 2-mercaptobenzimidazole sulfonic acids).

After development, the silver halide light-sensitive material is fixed in the present invention. Ordinary fixing compositions can be employed including thiosulfates, thiocyanates, and organic sulfur compounds which are known to have an effect as fixing agent. The fix solution may contain a water-soluble aluminum salt as a hardening agent.

The processing temperature in the process of the present invention is typically from 18°C to 50°C.

An automatic processor is preferably used for the photographic processing of the present invention. Even when the total processing time is in the range of from 90 seconds to 120 seconds,, negative photographic characteristics of super high contrast are obtained.

The developer for use in the present invention may contain the compound disclosed in JP-A-56-24347 as a silver stain inhibitor. Furthermore, the developer may contain the compound disclosed in JP-A-61-267759 as a resolution aid. Moreover, the developer may further contain the compound disclosed in JP-A-60-93433 or boron compounds disclosed in JP-A-62-186259.

The following examples are intended to illustrate the present invention but not to limit it in any way.

### EXAMPLE 1

A silver chloroiodobromide emulsion (containing 0.1 mol% silver iodide and 30 mol% silver bromide) was prepared using a double jet method as shown below. For preparing the silver chloroiodobromide emulsion, (NH₄)₃RhCl₆ was added to the aqueous halide solution (containing KBr, NaCℓ and KI)as a rhodium salt at a concentration of 5x10⁻⁶ mol/mol-Ag. K₃IrCl₆ was also added to the aqueous halide solution as an iridium salt at a concentration of 4x10⁻⁷ mol/mol-Ag.

The aqueous halide solution thus prepared and an aqueous silver nitrate solution were added to an aqueous gelatin solution and mixed for 60 minutes at 45°C to provide a mono-dispersed cubic grain size halide having a mean grain size of 0.25 µm. After washing the emulsion with water and desalting, 1x10⁻⁵ mol/mol-Ag of sodium thiosulfate and 1x10⁻⁵ mol/mol-Ag of potassium chloroaurate were added to the emulsion for gold sensitization. To the emulsion were further added 3x10⁻⁴ mol/mol-Ag of 1-(2-hydroxyethoxyethyl)-3-(pyridin-2-yl)-5-[(3-sulfobutyl-5-chloro-2-benzoxazolinidene)ethylidene]-2-thiohydantoin potassium salt as a sensitizing dye, 1.5 g of 4-hydroxy-6-methyl-1,3,3a,7-tetraazaindene as a stabilizer, 2 g of hydroquinone, 2 g of resorcin aldoxium, and 0.1 g of 1-phenyl-5-mercaptotetrazole each per mol of silver.

Furthermore, to the emulsion were added the compound of formula and saponin as coating aids, the compound of formula CH₂=CHSO₂CH₂CONH-(CH₂)ₙNHCOCH₂SO₂CH=CH₂ (n=2 or 3) as a hardening agent, sodium polystyrenesulfonate as a tackifier, and a dispersion of polyethyl acrylate as a latex polymer.

Moreover, to the emulsion were further added each of IX-9, IX-31, IX-20, IX-32, IX-34, and IX-35 as the hydrazine compound shown by formula (IX) and each of Ia-15 and Ib-7 as a nucleation accelerator as shown in Table 1 below to provide the silver halide emulsion.

A coating composition for a protective layer was composed of an aqueous gelatin solution containing gelatin, sodium dodecylbenzenesulfonate, colloidal silica, a dispersion of polyethyl acrylate, polymethyl methacrylate (matting agents), and sodium polystyrenesulfonate (tackifier).

The aforesaid emulsion and the coating composition for the protective layer were simultaneously coated on a transparent plastic film support at a gelatin coverage of 1.6 g/m² for the protective layer and a silver coverage of 3.6 g/m² for the emulsion layer.

Each sample thus prepared was exposed to tungsten light of 3200 K through a sensitometric optical wedge for 5 seconds, developed by developer (A) or (D) having the composition shown below for 30 seconds at 38°C, fixed, washed, and dried. An automatic processor FG-660F, made by Fuji Photo Film Co., Ltd. was used for the development processing.

| Composition of Developer (A) | |
|---|---|
| Hydroquinone | 35.0 g |
| N-Methyl-p-aminophenol $\frac{\text{1}}{\text{2}}$sulfate | 0.8 g |
| Sodium hydroxide | 9.0 g |
| Potassium tertiary phosphate | 74.0 g |
| Potassium sulfite | 90.0 g |
| Ethylenediaminetetraacetic acid di-sodium salt | 1.0 g |
| Potassium bromide | 3.0 g |
| 5-Methylbenzotriazole | 0.6 g |
| 3-Diethylamino-1-propanol | 15.0 g |
| Water to make | 1 liter |
| pH | 11.6 |

Developer (D) was prepared by adding acetic acid to developer (A) reducing the pH to 10.4.

Then, the $\overline{\text{G}}$ value of each sample thus processed was measured and the results obtained are shown in Table 1.

The $\overline{\text{G}}$ value is calculared by the equation $\overline{\text{G}}$=[3.0-0.3]/ΔlogE wherein ΔlogE is the difference in the exposure amounts (logE) necessary to attain the densities of 3.0 and 0.3, respectively.

Also, after placing 1 liter of each of the developers (A) and (D) in a one liter beaker and aged at room temperature and open to air for one week, the aforesaid sample was processed by the developer as described above and the $\overline{\text{G}}$ value was measured. The results are also shown in Table 1.

From the results shown in Table 1, it can be seen that by using the nucleation accelerator of the present invention, the $\overline{\text{G}}$ value is above 10 even at low developer pH-range as claimed . Also, development processing is stable as shown by the small difference in $\overline{\text{G}}$ value when using 1 week old developer.

### EXAMPLE 2

Developers (B), (C), (D), (E), (F), and (G) were prepared having the same composition as the developer in Example 1 except that the pH value was adjusted as shown in Table 2. Light-sensitive film prepared as in Sample No. 9 of Example 1 was processed using the developer of Example 1, as adjusted for pH, and the $\overline{\text{G}}$ value was then measured. The results are shown in Table 2. After placing one liter of each of the developers (A) to (G) in a one liter beaker and allowing to age at room temperature and open to air for one week, the light-sensitive film was processed using the one week old developer and the $\overline{\text{G}}$ value was measured. The results are also shown in Table 2.

**Table 2**

| | | $\overline{\text{G}}$ | |
|---|---|---|---|
| Developer | pH | Directly after Developer Preparation | Developer Aged 1 Week |
| (A) | 11.6 | 38 | 18 |
| (B) | 11.0 | 30 | 28 |
| (C) | 10.8 | 25 | 23 |
| (D) | 10.4 | 20 | 19 |
| (E) | 10.0 | 15 | 14 |
| (F) | 9.8 | 10 | 10 |
| (G) | 9.5 | 7 | 7 |
| - Developers (A) (B), (C) and (G):: For comparison - Developers (D) to (F):: For this invention | | | |

From the results in Table 2, it can be seen that by using the compounds of the present invention, a super high contrast value of at least a $\overline{\text{G}}$ of 10 is obtained and the $\overline{\text{G}}$ value remains stable, using aged developer, in the claimed pH range.

### EXAMPLE 3

The same procedure was followed as for Sample No. 9 in Example 1 except that each of Ia-16 and Ia-21 was added in place of Ia-15 to prepare Sample Nos. 26 and 27. Each sample was processed as in Example 1 and the $\overline{\text{G}}$ value was measured. The results are shown in Table 3.

**Table 3**

| | $\overline{\text{G}}$ | | $\overline{\text{G}}$ | |
|---|---|---|---|---|
| | Fresh Developer | | After 1 Week Developer | |
| Sample No. | pH 11.6 | pH 10.4 | pH 11.6 | pH 10.4 |
| | (A) | (D) | (A) | (D) |
| 26 | 35 | 18 | 15 | 17 |
| 27 | 32 | 15 | 12 | 14 |

From the results above, it can be seen that by using the compounds in the present invention, a super high contrast of $\overline{\text{G}}$ greater than 10 is obtained in the claimed pH-range and processing stability is maintained in the case of using the developer in the claimed pH-range.

### EXAMPLE 4

Developers (A), (B), (C), (D), (E), (F), and (G) were prepared as in Example 2. Also, by following the same procedure as Sample 23 in Example 1, a light-sensitive material was prepared, processed as in Example 1 using the developers (A) to (G) and the $\overline{\text{G}}$ value was measured. The results are shown in Table 4. Also, after placing one liter of each of the developers (A) to (G) in a one liter beaker and exposing the developer to air at room temperature for one week, the samples were processed as above using the developers (A) to (G) and the $\overline{\text{G}}$ value was measured. The results are shown in Table 4.

**Table 4**

| | | $\overline{\text{G}}$ | |
|---|---|---|---|
| Developer | pH | Fresh | After one week |
| (A) | 11.6 | 34 | 15 |
| (B) | 11.0 | 30 | 28 |
| (C) | 10.8 | 25 | 23 |
| (D) | 10.4 | 18 | 16 |
| (E) | 10.0 | 15 | 14 |
| (F) | 9.8 | 10 | 10 |
| (G) | 9.5 | 7 | 7 |
| - Developers (A) (B), (C) and (G):: For Comparison. - Developers (D) to (F):: For the Invention. | | | |

From the results shown above, it can be seen that by using the compounds in this invention, a super high contrast of $\overline{\text{G}}$ at least 10 is obtained, and the $\overline{\text{G}}$ value remains stable, using aged developer, in the claimed pH range.

### EXAMPLE 5

By following the same procedure as Sample No. 23 in Example 1 except that each of Ib-10 and Ib-31-was used in place of Ib-7 as the nucleating accelerator, Sample Nos. 28 and 29 were prepared. Each sample was processed as in Example 1 and the $\overline{\text{G}}$ value was measured. The results are shown in Table 5. Also, the developer was aged for one week as in Example 1, each sample was processed using the developers (A) and (B), and the $\overline{\text{G}}$ value was measured. The results are shown in Table 5.

**Table 5**

| | $\overline{\text{G}}$ | | $\overline{\text{G}}$ | |
|---|---|---|---|---|
| Sample No. | Fresh | | After 1 Week | |
| | (A) | (B) | (A) | (B) |
| 28 | 30 | 17 | 14 | 16 |
| 29 | 28 | 14 | 12 | 13 |

As shown in the above results, it can be seen that by using the compounds of the present invention, super high contrast of $\overline{\text{G}}$ value greater than 10 is obtained, and the $\overline{\text{G}}$ value remains stable and stability can be kept when using a developer in the claimed pH-range.

While the invention has been described in detail and with reference to specific embodiments thereof, it will be apparent to one skilled in the art that various changes and modifications can be made therein without departing from the scope thereof.

## Claims

1. A process for forming super high contrast negative images, which comprises processing a super high contrast negative type silver halide photographic material comprising a support having thereon at least one layer, one of which must be a silver halide emulsion layer, said silver halide emulsion layer or other hydrophilic colloid layer containing at least one hydrazine derivative and at least one nucleation accelerator represented by following formula (Ia) or (Ib) with a developer having a pH of from 9.6 to less than 10.5;
M₁S(̵X)̵ₙA₃-B (Ib)
wherein Y represents a group adsorbing onto silver halide; A₁ represents a divalent linkage group composed of an atom or an atomic group selected from carbon, nitrogen, oxygen, and sulfur; A₂ represents a divalent linkage group; A₃ represents a linkage group composed of an atom or an atomic group selected from carbon, nitrogen, oxygen, and sulfur; B represents a substituted or unsubstituted amino group, an ammonium group, or a nitrogen-containing heterocyclic ring; X represents a divalent heterocyclic ring containing nitrogen, oxygen, selenium or sulfur; M₁ represents a hydrogen atom, an alkali metal, an alkaline earth metal, a quaternary ammonium salt, a quaternary phosphonium salt, an amidino group; m represents the integer of 1, 2 or 3; and n and p each represents 0 or the integer 1.

2. A process as in claim 1, wherein said Y absorbing group is a nitrogen-containing heterocyclic group such that said nucleation accelerator is represented by formula wherein Q represents an atomic group necessary for forming a 5- or 6-membered heterocyclic ring composed of members selected from carbon, nitrogen, oxygen and sulfur or the condensation product of said 5- or 6-membered ring with a carbon aromatic ring or a heteroaromatic ring; M₂ represents hydrogen, an alkali metal atom, an ammonium group or a group capable of being replaced with hydrogen or an alkali metal atom under alkali conditions; and e represents 0 or the integer 1.

3. A process as in claim 2, wherein said nitrogen-containing heterocyclic group comprises a substituted or unsubstituted indazole, benzimidazole, benzoriazole, benzoxazole, benzthiazole, imidazole, thiazole, oxazole, triazole, tetrazole, azaindene, pyrazole, indole, triazine, pyrimidine, pyridine or quinoline.

4. A process as in claim 2, wherein said M₂ releasing group is acetyl, cyanoethyl or methanesulfonylethyl.

5. A process as in claim 1, wherein said divalent linkage group A₁ is or a combination thereof with a straight chain or branched alkylene group wherein R₁, R₂, R₃, R₄, R₅, R₆, R₇, R₈, R₉ and R₁₀ each represents hydrogen, a substituted or unsubstituted alkyl group, a substituted or unsubstituted aryl group, a substituted or unsubstituted alkenyl group or a substituted or unsubstituted aralkyl group.

6. A process as in claim 1, wherein said divalent linkage group A₂ is a straight chain or branched alkylene group, a straight chain or branched alkenylene group, a straight chain or branched aralkylene group or a straight chain or branched arylene group.

7. A process as in claim 1, wherein said divalent heterocyclic ring X comprises a substituted or unsubstituted tetrazole, triazole, thiadiazole, oxadiazole, selenadiazole, imidazole, thiazole, oxazole, benzimidazole, benzthiazole, benzoxazole, benzselenazole or pyrimidine.

8. A process as in claim 1, wherein said divalent linkage group A₃ is or a combination thereof with a straight chain or branched alkylene group and/or a straght chain or branched alkinylene group wherein R₁, R₂, R₃, R₄, R₅, R₆, R₇, R₈, R₉ and R₁₀ each represents hydrogen, a substituted or unsubstituted alkyl group, a substituted or unsubstituted aryl group, a substituted or unsubstituted alkenyl group or a substituted or unsubstituted aralkyl group.

9. A process as in claim 1, wherein said B nitrogen-containing heterocyclic ring is imidazolyl, pyridyl or thiazolyl.

10. A process as in claim 2, wherein said nucleation accelerator is represented by the formula

11. A process as in claim 2, wherein said nucleation accelerator is represented by the formula

12. A process as in claim 2, wherein said nucleation accelerator is represented by the formula

13. A process as in claim 2, wherein said nucleation accelerator is represented by the formula wherein Z₁, Z₂, and Z₃ each represents (A₁)̵ₚA₂-B or a halogen atom, an alkoxy group having from 1 to 20 carbon atoms, a hydroxy group, a hydroxyamino group or a substituted or unsubstituted amino group provided that at least one of Z₁, Z₂, and Z₃ is (A₁)̵ₚA₂-B.

14. A process as in claim 1, wherein said hydrazine derivative is represented by the formula R₂₁-NHNH-CHO wherein R₂₁ is an aliphatic group having from 1 to 30 carbon atoms or an aromatic group comprising a monocyclic or dicyclic aryl group, unsaturated heterocyclic group or the condensation product of the unsaturated heterocyclic group with the monocyclic or dicyclic aryl group.

15. A process as in claim 1, wherein said nucleation accelerator of formula (Ia) is added in an amount of from 5 mg/m² to 500 mg/m² to said photographic material.

16. A process as in claim 1, wherein said nucleation accelerator of formula (Ib) is added in an amount of from 1 mg/m² to 250 mg/m² to said photographic material.

17. A Process as in claim 1, wherein said hydrazine derivative is added in an amount of from 1 mg/m² to 300 mg/m².

18. A process as in claim 1, wherein said developer contains sulfite ion at a concentration of at least 0.15 mol/liter.

## Patentansprüche

1. Verfahren zur Bildung von Negativbildern mit superhohem Kontrast, umfassend das Verarbeiten eines photographischen Silberhalogenidnegativmaterials, umfassend einen Träger mit darauf wenigstens einer Schicht, wobei wenigstens eine davon eine Silberhalogenidemulsionsschicht sein muß, und die Silberhalogenidemulsionsschicht oder andere hydrophile Kolloidschicht wenigstens ein Hydrazinderivat und wenigstens einen durch folgende Formel (Ia) oder (Ib) dargestellten Keimbildungsbeschleuniger enthält, mit einem Entwickler mit einem pH von 9,6 bis weniger als 10,5
M₁S(̵X)̵ₙA₃-B (Ib)
worin bedeuten:
Y eine auf Silberhalogenid adsorbierende Gruppe; A₁ eine zweiwertige Verknüpfungsgruppe, gebildet aus einem Atom oder einer Atomgruppe, ausgewählt aus Kohlenstoff, Stickstoff, Sauerstoff und Schwefel; A₂ eine zweiwertige Verknüpfungsgruppe; A₃ eine Verknüpfungsgruppe, gebildet aus einem Atom oder einer Atomgruppe, ausgewählt aus Kohlenstoff, Stickstoff, Sauerstoff und Schwefel; B eine substituierte oder nicht-substituierte Aminogruppe, eine Ammoniumgruppe oder einen Stickstoff enthaltenden heterocyclischen Ring; X einen zweiwertigen heterocyclischen Ring, enthaltend Stickstoff, Sauerstoff, Selen oder Schwefel; M₁ ein Wasserstoffatom, ein Alkalimetall, ein Erdalkalimetall, ein quaternäres Ammoniumsalz, ein quaternäres Phosphoniumsalz, eine Amidinogruppe; m die ganze Zahl 1, 2 oder 3; und n und p jeweils 0 oder die ganze Zahl 1.

2. Verfahren nach Anspruch 1, worin die absorbierende Gruppe Y eine Stickstoff enthaltende heterocyclische Gruppe ist, derart, daß der Keimbildungsbeschleuniger durch die Formel dargestellt wird,
worin bedeuten:
Q eine Atomgruppe, welche notwendig ist zur Bildung eines 5- oder 6-gliedrigen heterocyclischen Rings, zusammengesetzt aus Bestandteilen, ausgewählt aus Kohlenstoff, Stickstoff, Sauerstoff und Schwefel, oder das Kondensationsprodukt des 5- oder 6-gliedrigen Rings mit einem aromatischen Kohlenstoffring oder einem heteroaromatischen Ring; M₂ Wasserstoff, ein Alkalimetallatom, eine Ammoniumgruppe oder eine Gruppe, die durch Wasserstoff oder ein Alkalimetallatom unter alkalischen Bedingungen ersetzt werden kann; und 1 0 oder die ganze Zahl 1.

3. Verfahren nach Anspruch 2, worin die Stickstoff enthaltende heterocyclische Gruppe ein substituiertes oder nicht-substituiertes Indazol, Benzimidazol, Benzotriazol, Benzoxazol, Benzthiazol, Imidazol, Thiazol, Oxazol, Triazol, Tetrazol, Azainden, Pyrazol, Indol, Triazin, Pyrimidin, Pyridin oder Chinolin umfaßt.

4. Verfahren nach Anspruch 2, worin die M₂-Freisetzungsgruppe Acetyl, Cyanoethyl oder Methansulfonylethyl ist.

5. Verfahren nach Anspruch 1, worin die zweiwertige Verknüpfungsgruppe A₁ oder eine Kombination davon
mit einer geradkettigen oder verzweigtkettigen Alkylengruppe ist, worin R₁, R₂, R₃, R₄, R₅, R₆, R₇, R₈, R₉ und R₁₀ jeweils Wasserstoff, eine substituierte oder nicht-substituierte Alkylgruppe, eine substituierte oder nicht-substituierte Arylgruppe, eine substituierte oder nicht-substituierte Alkenylgruppe oder eine substituierte oder nicht-substituierte Aralkylgruppe bedeuten.

6. Verfahren nach Anspruch 1, worin die zweiwertige Verknüpfungsgruppe A₂ eine geradkettige oder verzweigte Alkylengruppe, eine geradkettige oder verzweigte Alkenylengruppe, eine geradkettige oder verzweigte Aralkylengruppe oder eine geradkettige oder verzweigte Arylengruppe ist.

7. Verfahren nach Anspruch 1, worin der zweiwertige heterocyclische Ring X ein substituiertes oder nicht-substituiertes Tetrazol, Triazol, Thiadiazol, Oxadiazol, Selenadiazol, Imidazol, Thiazol, Oxazol, Benzimidazol, Benzthiazol, Benzoxazol, Benzselenazol oder Pyrimidin umfaßt.

8. Verfahren nach Anspruch 1, worin die zweiwertige Verknüpfungsgruppe A₃ oder eine Kombination davon
mit einer geradkettigen oder verzweigten Alkylengruppe und/oder einer geradkettigen oder verzweigten Alkinylengruppe ist, worin R₁, R₂, R₃, R₄, R₅, R₆, R₇, R₈, R₉ und R₁₀ jeweils Wasserstoff, eine substituierte oder nicht-substituierte Alkylgruppe, eine substituierte oder nicht-substituierte Arylgruppe, eine substituierte oder nicht-substituierte Alkenylgruppe oder eine substituierte oder nicht-substituierte Aralkylgruppe bedeuten.

9. Verfahren nach Anspruch 1, worin der Stickstoff enthaltende heterocyclische Ring B Imidazolyl, Pyridyl oder Thiazolyl ist.

10. Verfahren nach Anspruch 2, worin der Keimbildungsbeschleuniger durch die Formel dargestellt ist.

11. Verfahren nach Anspruch 2, worin der Keimbildungsbeschleuniger durch die Formel dargestellt ist.

12. Verfahren nach Anspruch 2, worin der Keimbildungsbeschleuniger durch die Formel dargestellt ist.

13. Verfahren nach Anspruch 2, worin der Keimbildungsbeschleuniger durch die Formel dargestellt ist, worin Z₁, Z₂ und Z₃ jeweils (A₁)̵ₚA₂-B oder ein Halogenatom, eine Alkoxygruppe mit 1 bis 20 Kohlenstoffatomen, eine Hydroxygruppe, eine Hydroxyaminogruppe oder eine substituierte oder nicht-substituierte Aminogruppe bedeuten, mit der Maßgabe, daß wenigstens eines von Z₁, Z₂ und Z₃ (A₁)̵ₚA₂-B ist.

14. Verfahren nach Anspruch 1, worin das Hydrazinderivat durch die Formel R₂₁-NHNH-CHO dargestellt ist, worin R₂₁ eine aliphatische Gruppe mit 1 bis 30 Kohlenstoffatomen oder eine aromatische Gruppe, umfassend eine monocyclische oder dicyclische Arylgruppe, ungesättigte heterocyclische Gruppe oder das Kondensationsprodukt der ungesättigten heterocyclischen Gruppe mit der monocyclischen oder dicyclischen Arylgruppe, ist.

15. Verfahren nach Anspruch 1, worin der Keimbildungsbeschleuniger der Formel (Ia) in einer Menge von 5 mg/m² bis 500 mg/m² zu dem photographischen Material zugegeben wird.

16. Verfahren nach Anspruch 1, worin der Keimbildungsbeschleuniger der Formel (Ib) in einer Menge von 1 mg/m² bis 250 mg/m² zu dem photographischen Material zugegeben wird.

17. Verfahren nach Anspruch 1, worin das Hydrazinderivat in einer Menge von 1 mg/m² bis 300 mg/m² zugegeben wird.

18. Verfahren nach Anspruch 1, worin der Entwickler Sulfitionen mit einer Konzentration von wenigstens 0,15 Mol/l enthält.

## Revendications

1. Procédé pour former des images négatives à ultra-haut contraste, qui comprend le traitement d'un matériau photographique à l'halogénure d'argent du type négatif à ultra-haut contraste comprenant un support portant au moins une couche, dont l'une doit être une couche d'émulsion d'halogénure d'argent, ladite couche d'émulsion d'halogénure d'argent ou une autre couche colloïdale hydrophile contenant au moins un dérivé d'hydrazine et au moins un accélérateur de nucléation représenté par la formule (Ia) ou (Ib) suivante avec un révélateur ayant un pH de 9,6 à moins de 10,5
M₁S(̵X)̵ₙ-A₃-B (Ib)
dans lesquelles Y représente un groupe s'adsorbant sur l'halogénure d'argent ; A₁ représente un chaînon de liaison divalent composé d'un atome ou d'un groupe atomique choisi parmi le carbone, l'azote, l'oxygène et le soufre ; A₂ représente un chaînon de liaison divalent ; A₃ représente un chaînon de liaison divalent composé d'un atome ou d'un groupe atomique choisi parmi le carbone, l'azote, l'oxygène et le soufre ; B représente un groupe amino substitué ou non, un groupe ammonium ou un hétérocycle azoté ; X représente un hétérocycle divalent contenant de l'azote, de l'oxygène, du sélénium ou du soufre ; M₁ représente un atome d'hydrogène, un atome de métal alcalin, un atome de métal alcalino-terreux, un sel d'ammonium quaternaire, un sel de phosphonium quaternaire ou un groupe amidino ; m représente 1, 2 ou 3 ; et n et p représentent chacun 0 ou 1.

2. Procédé selon la revendication 1, dans lequel ledit groupe adsorbable Y est un groupe hétérocyclique azoté tel que ledit accélérateur de nucléation est représenté par la formule dans laquelle Q représente un groupe atomique nécessaire pour former un hétérocycle à 5 ou 6 chaînons composé d'éléments choisis parmi le carbone, l'azote, l'oxygène et le soufre ou le produit de condensation dudit cycle à 5 ou 6 chaînons avec un noyau aromatique carboné ou un noyau hétéroaromatique ; M₂ représente l'hydrogène, un atome de métal alcalin, un groupe ammonium ou un groupe remplaçable par l'hydrogène ou par un atome de métal alcalin en conditions alcalines ; et ℓ représente 0 ou 1.

3. Procédé selon la revendication 2, dans lequel ledit groupe hétérocyclique azoté comprend un noyau indazole, benzimidazole, benzotrimole, benzoxazole, benzothiazole, imidazole, thiazole, oxazole, triazole, tétrazole, azaindène, pyrazole, indole, triazine, pyrimidine, pyridine ou quinoléine substitué ou non.

4. Procédé selon la revendication 2, dans lequel ledit groupe séparable M₂ est un groupe acétyle, cyanoéthyle ou méthanesulfonyléthyle.

5. Procédé selon la revendication 1, dans lequel ledit chaînon de liaison divalent A1 est ou une de leurs combinaisons avec un groupe alkylène à chaîne droite ou ramifiée, dans lesquels R₁, R₂, R₃, R₄, R₅, R₆, R₇, R₈, R₉ et R₁₀ représentent chacun l'hydrogène, un groupe alkyle substitué ou non, un groupe aryle substitué ou non, un groupe alcényle substitué ou non ou un groupe aralkyle substitué ou non.

6. Procédé selon la revendication 1, dans lequel ledit chaînon de liaison divalent A₂ est un groupe alkylène à chaîne droite ou ramifiée, un groupe alcénylène à chaîne droite ou ramifiée, un groupe aralkylène à chaîne droite ou ramifiée, ou un groupe arylène à chaîne droite ou ramifiée.

7. Procédé selon la revendication 1, dans lequel ledit noyau hétérocyclique divalent X comprend un noyau tétrazole, triazole, thiadiazole, oxadiazole, sélénadiazole, imidazole, thioazole, oxazole, benzimidazole, benzothiazole, benzoxazole, benzosélénazole ou pyrimidine substitué ou non.

8. Procédé selon la revendication 1, dans lequel ledit chaînon de liaison divalent A3 est ou une de leurs combinaisons avec un groupe alkylène à chaîne droite ou ramifiée, et/ou un groupe alcynylène à chaîne droite ou ramifiée, où R₁, R₂, R₃, R4, R₅, R₆, R₇, R₈, R₉ et R₁₀ représentent chacun l'hydrogène ou un groupe alkyle substitué ou non , un groupe aryle substitué ou non, un groupe alcényle substitué ou non ou un groupe aralkyle substitué ou non.

9. Procédé selon la revendication 1, dans lequel ledit noyau hétérocyclique azoté B est un noyau imidazolyle, pyridyle ou thiazolyle.

10. Procédé selon la revendication 2, dans lequel ledit accélérateur de nucléation est représenté par la formule

11. Procédé selon la revendication 2, dans lequel ledit accélérateur de nucléation est représenté par la formule

12. Procédé selon la revendication 2, dans lequel ledit accélérateur de nucléation est représenté par la formule

13. Procédé selon la revendication 2, dans lequel ledit accélérateur de nucléation est représenté par la formule dans laquelle Z₁, Z₂ et Z₃ représentent chacun (A₁)̵ₚA₂-B ou un atome d'halogène, un groupe alcoxy en C₁-C₂₀, un groupe hydroxyle, un groupe hydroxylamino ou un groupe amino substitué ou non pourvu que l'un au moins des restes Z₁, Z₂ et Z₃ soit (A₁)̵ₚA₂-B.

14. Procédé selon la revendication 1, dans lequel ledit dérivé d'hydrazine est représenté par la formule R₂₁-NHNH-CHO dans laquelle R₂₁ est un groupe aliphatique en C₁-C₃₀ ou un groupe aromatique comprenant un groupe aryle monocyclique ou dicyclique, un groupe hétérocyclique insaturé ou un groupe hétérocyclique insaturé condensé avec le groupe aryle monocyclique ou dicyclique.

15. Procédé selon la revendication 1, dans lequel ledit accélérateur de nucléation de formule (Ia) est ajouté audit matériau photographique en quantité de 5 à 500 mg/m².

16. Procédé selon la revendication 1, dans lequel ledit accélérateur de nucléation de formule (Ib) est ajouté audit matériau photographique en quantité de 1 à 250 mg/m².

17. Procédé selon la revendication 1, dans lequel ledit dérivé d'hydrazine est ajouté en quantité de 1 à 300 mg/m².

18. Procédé selon la revendication 1, dans lequel ledit révélateur contient des ions sulfites à une concentration d'au moins 0,15 mol/l.
